

## UNITED STATES PATENT OFFICE

2,110,891

CORROSION-RESISTANT AND COLD WORK-  
ABLE MOLYBDENUM STEELHeinrich Reitz, Bitterfeld, and Erich Hengler and  
Alfred Bütinghaus, Wetzlar, GermanyNo Drawing. Application May 7, 1936, Serial  
No. 78,316. In Germany May 7, 1935

5 Claims. (Cl. 75—126)

The present invention relates to steels capable of resisting attack by corrosive media including aqueous solutions of chlorine, hypochlorous acid and their salts.

5 One of the chief problems with which the present day metallurgists are faced is a meeting of the demand by the chemical arts for steels which will withstand corrosive chemicals and still be capable of being mechanically worked. This 10 problem is particularly onerous as regards those industries which employ solutions of chlorine-containing substances, since, as is known, ferrous metals are very susceptible to attack by these substances. In fact, screens and the like used 15 in filtering apparatus in the manufacture of hypochlorites, when made of so-called stainless steel, are so vigorously attacked that their utility is completely impaired after only short periods of service.

20 Chromium is one of the alloying elements which is most commonly employed in steels designed for use in chemical apparatus. This element has the function, among others, of improving the corrosion resistance of the steel. Molybdenum has recently come into rather extended 25 use, usually with chromium as an agent for increasing or imparting corrosion resistance. Neither this element nor chromium, nor both together, however, is capable of giving steels this 30 property to an extent sufficient to withstand the attack of different chemicals especially solutions of chlorine-containing substances. Moreover, molybdenum, when used in large amounts, has a marked tendency to render steels brittle thereby 35 impairing their capability of being mechanically worked in the cold, that is cold rolled, cold drawn and cold hammered. Any increase in corrosion 40 resistance resulting from the use of large proportions of molybdenum is, therefore, offset by a decrease in the mechanical cold workability of the steels.

The purpose of this invention is to provide a chromium-molybdenum low-carbon steel which will be resistant to attack by aqueous solutions 45 of chlorine, hypochlorous acid, their salts and the like, and at the same time will possess the desired mechanical properties of being cold rolled, cold drawn, cold hammered and the like to a high degree.

50 We have discovered that if there is included in low carbon-chromium-molybdenum steels an alloying ingredient capable of forming carbides, in such quantities that after a fixing of the free carbon as carbide there remains sufficient of the 55 ingredients to form mixed crystals with the other alloying ingredients, steels of a resistance to chlorine-containing solutions which could not be foreseen are obtained. The alloying ingredient that we have found most suitable for use and 60 which we therefore prefer, is titanium. How-

ever, other elements may be used in lieu of titanium with satisfactory results. Thus, such carbide-forming elements as vanadium, tantalum, uranium, niobium, cerium, boron, zirconium and tungsten may be used as substitutes for titanium. 5

As previously noted, we have found it preferable in making up our alloys to maintain a low content of carbon, that is less than about .5%. The chromium content of the alloys should range between about 12 and 30%, preferably 10 between about 20 and 30%. The molybdenum content may be as high as 5% and should exceed about 1.5%. The titanium or other carbide forming element should be present in an amount of from about .5 to 3.5%. The addition of small 15 amounts of manganese and silicon are also to be recommended. Thus the steel preferably contains from about .3 to about .6% of manganese and less than .5% of silicon. The balance of the 20 steel is iron with the usual negligible quantities of impurities generally present in stainless steels.

These steels, especially when prepared with titanium, not only are remarkably resistant to corrosion by chlorine-containing solutions but also possess the property of being cold rolled, 25 cold hammered and cold drawn. An estimate of their resistance to corrosion may be gleaned from the fact that said steels are capable of withstanding attack by the very corrosive calcium 30 hypochlorite solutions even at a temperature of 110° C. Said steels may, therefore, be employed for all purposes where steels of these properties are required. Thus they are admirably fitted for the manufacture of wire screens for filtering 35 chlorine- and hypochloride-containing mashes and lyes and perforated supporting discs for such filters as well as armatures, armature accessories, pumps, containers, valves, slide bars and the like which during use contact chlorine-containing 40 solutions.

The following illustrates typical alloys within the scope of our invention:

|                                                             |                     | Per cent |
|-------------------------------------------------------------|---------------------|----------|
| 1. Carbon                                                   | =less than-----     | 0.50     |
| Manganese                                                   | =-----0.30- 0.60    | 45       |
| Silicon                                                     | =less than-----0.50 |          |
| Chromium                                                    | =-----12.5-30.0     |          |
| Molybdenum                                                  | =-----1.50- 5.00    |          |
| Titanium                                                    | =-----0.50- 3.50    |          |
| Balance iron and negligible quantities of usual impurities. |                     | 50       |
| 2. Carbon                                                   | =less than-----0.10 |          |
| Manganese                                                   | =-----0.40- 0.60    | 55       |
| Silicon                                                     | =less than-----0.50 |          |
| Chromium                                                    | =-----16.0-18.0     |          |
| Molybdenum                                                  | =-----1.80- 2.40    |          |
| Titanium                                                    | =-----0.80- 1.20    |          |
| Balance iron and negligible quantities of usual impurities. |                     | 60       |

|     |                                                             | Per cent   |      |  |  |  |  |
|-----|-------------------------------------------------------------|------------|------|--|--|--|--|
| 3.  | Carbon                                                      | 0.20- 0.30 |      |  |  |  |  |
|     | Manganese                                                   | 0.40- 0.60 |      |  |  |  |  |
|     | Silicon                                                     | =less than | 0.50 |  |  |  |  |
| 5.  | Chromium                                                    | 23.0- 25.0 |      |  |  |  |  |
|     | Molybdenum                                                  | 2.80- 3.30 |      |  |  |  |  |
|     | Titanium                                                    | 1.80- 2.40 |      |  |  |  |  |
|     | Balance iron and negligible quantities of usual impurities. |            |      |  |  |  |  |
| 10. | 4. Carbon                                                   | 0.18- 0.22 |      |  |  |  |  |
|     | Manganese                                                   | 0.40- 0.60 |      |  |  |  |  |
|     | Silicon                                                     | =less than | 0.50 |  |  |  |  |
|     | Chromium                                                    | 27.0- 29.0 |      |  |  |  |  |
| 15. | Molybdenum                                                  | 1.60- 2.00 |      |  |  |  |  |
|     | Titanium                                                    | 1.20- 1.60 |      |  |  |  |  |
|     | Balance iron and negligible quantities of usual impurities. |            |      |  |  |  |  |
| 20. | 5. Carbon                                                   | =less than | 0.50 |  |  |  |  |
|     | Manganese                                                   | 0.40- 0.60 |      |  |  |  |  |
|     | Silicon                                                     | =less than | 0.50 |  |  |  |  |
|     | Chromium                                                    | 20.0- 30.0 |      |  |  |  |  |
|     | Molybdenum                                                  | 1.80- 4.00 |      |  |  |  |  |
|     | Titanium                                                    | 0.50- 3.50 |      |  |  |  |  |
| 25. | Balance iron and negligible quantities of usual impurities. |            |      |  |  |  |  |

rium, cerium, boron, zirconium or tungsten. However, when such metals are used in lieu of titanium, it is preferable to maintain the proportions of elements of Example 5.

Titanium has heretofore been used in steels but primarily for the purpose of effecting de-oxidation thereof. This use is in no way comparable to our use of titanium. On the contrary, the presence of titanium in our steels serves the purposes of augmenting the corrosion resistance of the steel imparted by the molybdenum and of preventing the molybdenum from destroying the desired mechanical properties of the steel such as its cold rollability, cold ductility and cold malleability. Thus, the steels have a much greater resistance to corrosion than could be imparted to them by molybdenum alone, and at the same time are capable of being mechanically worked in the cold despite the presence of substantial quantities of molybdenum.

The two fold function of the titanium in our steels is developed in the accompanying tables which compare the corrosion resistance and cold malleability of chromium-molybdenum steels with chromium-molybdenum-titanium steels.

## (1)

| 30 | C    | Mn        | Si     | Cr    | Mo  | Ti%   | Loss of weight in grams/sq. meter of surface in 1 hour |                                                                              |                                                                              | Depth in mm. in a foil 1 mm. in thickness acc. to Erichsen | 30 |
|----|------|-----------|--------|-------|-----|-------|--------------------------------------------------------|------------------------------------------------------------------------------|------------------------------------------------------------------------------|------------------------------------------------------------|----|
|    |      |           |        |       |     |       | Acetic acid conc. +5 gr. NaCl, temperature 90° C.      | 10% H <sub>2</sub> SO <sub>4</sub> +4% HNO <sub>3</sub> , temperature 90° C. | 20% H <sub>2</sub> SO <sub>4</sub> +4% HNO <sub>3</sub> , temperature 90° C. |                                                            |    |
| 35 | 0.10 | 0.40-0.60 | 0.30-1 | 14.92 | 2.0 | ----- | *                                                      | 10.5                                                                         | 2.3                                                                          | 7.3                                                        | 35 |
|    | 0.08 | 0.40-0.60 | 0.30-1 | 15.97 | 2.0 | 0.45  | 2.31                                                   | 1.265                                                                        | 0.001                                                                        | 10.85                                                      |    |
|    | 0.07 | 0.40-0.60 | 0.30-1 | 17.60 | 2.0 | 0.93  | 0.62                                                   | 1.152                                                                        | 0.000                                                                        | 10.40                                                      |    |
| 40 |      |           |        |       |     |       |                                                        |                                                                              |                                                                              | 40                                                         |    |
| 45 |      |           |        |       |     |       |                                                        |                                                                              |                                                                              | 45                                                         |    |

## (2)

| 50 | C    | Mn        | Si     | Cr    | Mo   | Ti%   | Loss of weight in grams/sq. meter of surface in 1 hour |                                                                   |                                                                                                    | Depth in mm. in a foil 1 mm. in thickness acc. to Erichsen | 50 |
|----|------|-----------|--------|-------|------|-------|--------------------------------------------------------|-------------------------------------------------------------------|----------------------------------------------------------------------------------------------------|------------------------------------------------------------|----|
|    |      |           |        |       |      |       | 10% H <sub>2</sub> SO <sub>4</sub> at 20° C.           | 20% H <sub>2</sub> SO <sub>4</sub> +4% HNO <sub>3</sub> at 20° C. | NaOCl solution containing 90 gms. of chlorine per lt. and 400 grams of CaCl <sub>2</sub> at 20° C. |                                                            |    |
| 55 | 0.27 | 0.40-0.60 | 0.30-1 | 24.83 | 2.0  | ----- | 10.5                                                   | 0.027                                                             | Strong pitting.                                                                                    | 6.5                                                        | 55 |
|    | 0.07 | 0.40-0.60 | 0.30-1 | 26.70 | 2.30 | ----- | 10.0                                                   | *                                                                 | Strong pitting.                                                                                    | 7.1                                                        |    |
|    | 0.20 | 0.40-0.60 | 0.30-1 | 26.28 | 1.88 | 1.39  | 0.00                                                   | 0.0058                                                            | No attack.                                                                                         | 7.5                                                        | 65 |
| 60 | 0.08 | 0.40-0.60 | 0.30-1 | 29.15 | 1.71 | 1.29  | 0.00                                                   | 0.0000                                                            | No attack.                                                                                         | 8.2                                                        |    |
| 65 | 0.27 | 0.40-0.60 | 0.30-1 | 26.28 | 4.00 | ----- | 4.5                                                    | *                                                                 | Pitting.                                                                                           | Not cold workable.                                         | 70 |
| 70 |      |           |        |       |      |       |                                                        |                                                                   |                                                                                                    |                                                            |    |

The titanium in any of these alloys may be replaced by vanadium, tantalum, uranium, nio-

The asterisks in the above tables indicate that the results were not ascertained with particular

ity since it was apparent from observation that the test pieces had suffered a very material decrease in weight, a fact which was to be expected at the outset.

5 For a full discussion of the Erichsen test referred to in the tables attention is directed to page 154 of "Enzyklopädie der technischen Chemie" by Ullmann, volume 4, 2nd edition.

What we claim is:

16 1. Cold ductile and cold malleable corrosion-resistant alloys for use in the manufacture of articles which require resistance to attack by aqueous solutions of chlorine, calcium hypochlorite and their salts, containing less than .5% of carbon, from about .3 to about .6% of manganese, less than about .5% of silicon, from about 12 to about 30% of chromium, from about 1.5 to about 5% of molybdenum, and from about .5 to about 3.5% of a carbide-forming element selected from 20 the class consisting of titanium and vanadium in an amount of about 6 to 12 times the amount of carbon present, the balance being iron with the usual impurities.

2. The alloy as defined in claim 1, wherein the 25 carbide-forming element is titanium.

3. Cold ductile and cold malleable corrosion-resistant alloys consisting of

|            | Per cent   |            |
|------------|------------|------------|
| Carbon     | =less than | 0,10       |
| Manganese  | =          | 0,40- 0,60 |
| Silicon    | =less than | 0,50       |
| Chromium   | =          | 16,0-18,0  |
| Molybdenum | =          | 1,80- 2,40 |
| Titanium   | =          | 0,80- 1,20 |

Balance iron and negligible quantities of usual impurities.

4. Cold ductile and cold malleable corrosion-resistant alloys consisting of

|            | Per cent   |            |
|------------|------------|------------|
| Carbon     | =-----     | 0,20- 0,30 |
| Manganese  | =-----     | 0,40- 0,60 |
| Silicon    | =less than | 0,50       |
| Chromium   | =-----     | 23,0-25,0  |
| Molybdenum | =-----     | 2,80- 3,30 |
| Titanium   | =-----     | 1,80- 2,40 |

Balance iron and negligible quantities of usual impurities.

5. Cold ductile and cold malleable corrosion-resistant alloys consisting of

|            | Per cent   |            |
|------------|------------|------------|
| Carbon     | =-----     | 0,18- 0,22 |
| Manganese  | =-----     | 0,40- 0,60 |
| Silicon    | =less than | 0,50       |
| Chromium   | =-----     | 27,0-29,0  |
| Molybdenum | =-----     | 1,60- 2,00 |
| Titanium   | =-----     | 1,20- 1,60 |

Balance iron and negligible quantities of usual impurities.

HEINRICH REITZ.

ERICH HENGLER.

ALFRED BÜTTINGHAUS.